

June 1, 1926.

1,586,887

G. W. ELMEN

INDUCTIVELY LOADING SIGNALING CONDUCTORS

Filed May 2, 1922

Fig. 1.



Fig. 2.



Inventor:

Gustaf W. Elmen.

by C. C. Sprague. Atty.

## UNITED STATES PATENT OFFICE.

GUSTAF W. ELMEN, OF LEONIA, NEW JERSEY, ASSIGNOR TO WESTERN ELECTRIC COMPANY, INCORPORATED, OF NEW YORK, N. Y., A CORPORATION OF NEW YORK.

## INDUCTIVELY LOADING SIGNALING CONDUCTORS.

Application filed May 2, 1922. Serial No. 557,928.

This invention relates to conductors for the transmission of electrical energy and more particularly to signaling conductors having an external layer of material of high permeability for the purpose of increasing the inductance.

One manner of increasing the inductance of a conductor employed for the transmission of alternating current is to wrap the conductor spirally with a layer of wire or tape of magnetic material. This method is known in the art as continuous inductive loading as distinguished from lump loading by means of coils distributed at intervals along the conductor. Until recently iron has been considered to be the only material suitable for continuous loading. It has been discovered however that a more suitable material may be produced in the form of an alloy of nickel and iron. When these two metals are in proper proportions and the alloy is given a proper heat treatment a material having a very high permeability at low magnetizing forces is obtained. This material is known as permalloy. In its preferred form it comprises 78½% nickel and 21½% iron. Other properties possessed by this alloy which increase its value as loading material are small hysteresis loss and high resistivity, both conductive to increasing the efficiency of the cable by lowering the effective resistance.

When it was attempted to employ this material in the form of a tape for continuously loading a conductor difficulties were encountered. It was found that if the permalloy tape is first heat-treated and then cooled and applied to the conductor internal stresses are set up by the bending of the tape, causing the permeability to be very materially lowered. This difficulty has been met in an entirely satisfactory manner according to this invention.

An object of this invention is to provide for the practical loading of a signaling conductor with magnetic material which requires heat treatment and whose characteristics are subject to undesired change under applied stresses.

A further object of the invention is to provide a method of applying magnetic loading material to an electrical conductor in a manner to prevent the setting up of deleterious stresses in the magnetic material during a subsequent heat treatment. More

specifically, the invention provides a method of applying loading material capable of possessing high permeability in a manner to avoid obtaining low and variable values of permeability.

The accompanying drawing shows, in Fig. 1, a conductor wrapped with magnetic tape and in Fig. 2 a furnace which is suitable for the heat treatment of the wrapped conductor.

It has been found desirable to employ a tape of a thickness not exceeding 9 or 10 mils and a width of 20 to 200 mils with conductors of the order of 100 to 200 mils in diameter. It is sometimes of advantage to use tape of only 2 or 3 mils thickness. These and other quantitative values mentioned in this specification are given by way of example only. It is to be understood that the invention is applicable under a wide range of conditions and the scope is defined only by the appended claims.

The ingredients of the magnetic alloy, permalloy for example, are first fused together in an induction furnace, then molded into the form of a bar or rod, and may then be worked down into the form of a wire of desired diameter. This process, as is usual, consists of successive drawings of the material until it acquires a certain degree of hardness, when it is annealed to soften it. The drawing process is then continued until it is again necessary to anneal. This cycle is repeated until the size of wire desired is obtained. If the loading material is to be in the form of tape, which is the preferred form, there is substituted for the drawing of the material during the last few cycles of operation a passing of it between rollers. A uniform width of tape may be obtained by trimming the edges.

To give the permalloy its desired characteristics including high permeability at small magnetizing forces it is necessary to heat-treat it. According to present practice this heat treatment comprises heating the tape to a temperature of about 850° C., maintaining it at that temperature for a few minutes to insure a uniform temperature throughout, then cooling slowly to a temperature of about 600 degrees, which is just above the critical or transition temperature of the alloy, that is the temperature at which the magnetic properties disappear on heating and reappear on cooling;

and finally cooling from that temperature more rapidly but at a definite rate dependent upon the ratio of nickel to iron in the alloy. This rate can be easily determined by trials. A convenient method of securing the desired rate of cooling has been found to be a rapid withdrawing of the material from the furnace when it has reached the temperature of 850° C. into a blast of air which is controlled to secure the desired rate of cooling. The necessary cooling will always be at a rate intermediate that required for annealing and that at which such strains would be set up as to lower the permeability below the desired value.

The magnetizing forces to which the loading material upon a signaling conductor is subjected are very small. They are of the order of 0.01 to 0.10 gauss. The permeability of permalloy at these small forces has been found to be from 10 to 20 times that of iron, that is from 3000 to 6000. The corresponding value for the best grades of iron is about 300. The permeability of this alloy may be reduced, however, to values of the order of 600 by the mere act of stretching the material. It would be impractical therefore to give the tape a final heat treatment before winding it upon the conductor. Such a process would so lower the permeability and make it vary so much from point to point that the loaded conductor would be of very inferior quality.

According to the present invention the above described difficulty is overcome by first placing the tape upon the conductor and then subjecting the conductor and tape to the same heat treatment. The tape is thus given its desired electrical characteristics after it is in its final shape and position. A further difficulty was encountered in the development of this process and an additional feature of this invention is the provision of additional steps in the process to overcome this difficulty. During the cooling subsequent to the heating, the temperature of the tape is lowered more quickly than that of the copper conductor, which results in permanent stresses introduced in the loading material due to the difference in the rates of contraction of the conductor and the loading material. The set thus given the material may result in a greatly reduced permeability. According to this invention this difficulty has been overcome by hardening the tape material before its application to the conductor, and applying only a moderate tension to the tape during the process of winding. The tape then appears to be rather firmly wound upon the conductor, but in fact there is sufficient spacing between the two to permit of the above mentioned difference in the rates of contraction of the conductor and

tape without producing a set in the tape. The value of the tension applied to the tape during winding should be no less or only very slightly less than that necessary to prevent this deleterious effect. Nine or ten ounces has been found to be a suitable value of tension in certain specific cases, but the best value must be determined by trial in each case.

The hardening of the wire or tape referred to in the preceding paragraph is accomplished by regulating the amount of reduction in diameter or thickness during the last stage of drawing or rolling. For example, a tape to have a thickness of 4 mils may have its final stage of annealing when it is 6 mils thick.

Referring to the drawing the tape 10 is shown as wound spirally upon the signaling conductor 11 with the edges of the adjacent turns in contact. If it were for any reason desired, the turns could be out of contact or could overlap. The preferred form is as shown. After the winding process the heat treatment may be effected by drawing the conductor lengthwise through the furnace shown in Fig. 2 which is maintained at a temperature of 850 degrees centigrade. This is a muffle furnace with the heating elements 20 between the fire clay muffle 21 and the fire brick 22. Around the fire brick is a sheet iron outer wall. The iron tube 23 has a copper lining 24 of inside diameter of little over  $\frac{1}{2}$  inch. This extends across the furnace and may project beyond the furnace walls at each end. The length of the pass through the furnace is about 2 feet and the rate of movement of the conductor therethrough is about  $\frac{3}{4}$  feet per minute. As the taped conductor passes through the furnace it is cooled by the air outside which is about 20 degrees centigrade. Under the conditions and for the dimensions described this gives a proper rate of cooling. For a different rate of withdrawal of the taped conductor from the furnace it may be advantageous to employ the cooling air-blast 25.

Although this process has been invented in connection with the development of permalloy loading it is obviously of more general application. The preferred material for loading is permalloy containing 78½% of nickel and 21½% of iron, but the wire or tape may be of any material which requires heat-treatment and which has a characteristic subject to undesired change under applied stress. Among the loading materials which could be used are iron-nickel alloys in which the percentage varies quite widely from that herein mentioned and also alloys containing other ingredients in addition to iron and nickel—for example, chromium, which may be added to increase the resistivity.

The process described is also applicable to the case where several layers of wire or tape are used, the adjacent layers of wire or tape being applied to the conductor in either the same or in opposite directions. It is sometimes advisable to use two or more layers of wire or tape, rather than one layer of greater thickness, to reduce the eddy current losses.

10 In a broad aspect the invention is not limited to the use of wire or tape. The layer of loading material may be applied in some other manner, but it must be in such a way that strains will not be set up in it during cooling of the loaded conductor after the final application of heat.

It is within the scope of the invention to operate the furnace in which the loaded conductor is heated at a temperature varying considerably from that mentioned above. It is necessary that the heating above the magnetic transition temperature be of a nature to render the structure of the alloy uniform throughout. This may be done by maintaining for a considerable time a temperature slightly above the transition point; but the process will be materially hastened if a very much higher temperature is maintained, and no harm will result. In order to maintain uniform structure throughout the material, it is also highly desirable to keep the conductor straight both while being heated and cooled. It is not completely understood what action takes place during the heating process, but there is evidence to support the view that a recrystallization of portions of the alloy, in which crystals were broken down by previous working of the material, takes place.

40 There is mentioned above the difference in rates of contraction of the loading tape and the copper conductor during the cooling stage of the heat treatment as a cause of low permeability of the heat treated loaded conductor. It may be that the contact of the hot loading material and conductor under pressure resulting from the difference in rates of contraction of the two materials causes them to adhere or weld at numerous points so that further cooling results in strains set up between these points. There is evidence to support this view. It may be too that the hardness of the magnetic material is per se of advantage in obtaining maximum benefit from the heat treatment as well as being a practical way of obtaining the desired looseness. Other explanations for the observed effect have been made, but, whatever the cause, the effect is substantially overcome or prevented by this invention.

For a more detailed account of the properties of the loading material described herein, see application of G. W. Elmen Serial No. 473,877, filed May 31, 1921. A complete

disclosure of the advantages of this material as a loading material for submarine telegraph cables is made in the application of O. E. Buckley, Serial No. 492,725, filed August 16, 1921.

70

What is claimed is:

1. The method of loading a signaling conductor with magnetic alloy the permeability of which varies materially when the alloy is strained, which comprises forming a layer of said alloy about the conductor so that the space within the loading layer is not completely occupied by the material of the conductor, and subjecting the loaded conductor to heat treatment, the layer being so formed that the conductor has room for expansion during the heat treatment.

75

2. The method of producing a signaling conductor loaded with magnetic material which requires heat treatment to give it high permeability and the permeability of which is sensitive to strains, which comprises forming a layer of said material about the conductor, so that the space within the layer is not completely occupied by the material of the conductor and subjecting the loaded conductor to the said heat treatment by passing it through a furnace and then through a cooling medium without bringing the conductor forcibly in contact with the inner surface of the loading layer.

80

3. The method of loading a signaling conductor the wire or tape of a material which requires heat treatment for maximum permeability, which comprises winding the wire or tape spirally upon the conductor before the final heat treatment and in such manner that the layer of loading material when cold will fit the conductor closely enough to prevent material slipping upon the conductor during the handling of the latter but not so tightly that the conductor during cooling after the final application of heat will interfere with contraction of the loading material when the cooling is at a proper rate to give high permeability, heating the wrapped conductor above the critical temperature of the magnetic material, and cooling it at a rate to give said material high permeability when cold.

90

4. The method of producing a signaling conductor loaded with magnetic material which requires a heat treatment for the development of high permeability therein and the permeability of which is sensitive to strain, which comprises forming a layer of the material about the conductor so that the space within the layer is not completely occupied by the material of the conductor, passing the loaded conductor through a furnace and a cooling medium in succession, and maintaining in a substantially straight condition that portion of the conductor which is being heated and cooled.

95

5. The method of loading a signaling con-

100

105

110

115

120

125

130

- 4
- ductor with magnetic material in the form of a wire or tape which comprises wrapping the wire or tape spirally about the conductor under a moderate tension, heating the wound conductor above the critical temperature of the magnetic material and subsequently cooling it at a rate necessary to give said material high permeability when cold, said tension being great enough to cause the wire or tape to lie in place while the conductor is handled but not great enough to cause such a close fit that the conductor will be brought forcibly in contact with the tape during said cooling process.
15. 6. The method of loading a signaling conductor with magnetic material in the form of a wire or tape which comprises regulating the hardness of the wire or tape, wrapping the cold wire or tape spirally about the conductor under a moderate tension, heating the wound conductor above the critical temperature of the magnetic material, and then cooling it, said tension being great enough to prevent the turns of the wire or tape from overlapping or materially slipping during subsequent handling of the conductor, but not so great that the conductor when undergoing said cooling process will set up a tension in the tape.
20. 7. The method of loading a signaling conductor with magnetic material in the form of wire or tape, which comprises wrapping the wire or tape spirally around the conductor under a moderate tension, heating the wound conductor well above the critical temperature of the magnetic material, cooling it slowly to a point just above the critical temperature and completing the cooling more rapidly at a predetermined rate whereby said material is given high permeability when cold, said tension being great enough to prevent the tape from subsequently overlapping or materially slipping during handling of the conductor but not great enough to cause such a close fit that the conductor will set up a tension in the magnetic material during said cooling process.
25. 8. The method of loading a signaling conductor with magnetic material which requires heat-treatment for maximum permeability, which comprises surrounding the conductor with a layer of the magnetic material fitting the conductor loosely enough at least to prevent the conductor during the cooling after the final application of heat from interfering with contraction of the loading material when the cooling is at a proper rate to give high permeability, heating the loaded conductor above the magnetic transition temperature of the loading material, and cooling it at said rate.
30. 9. The combination with a copper conductor of a layer of magnetic material thereabout which is capable of having developed therein high permeability at magnetizing forces encountered in signaling, but which has to be heat treated after being applied to the conductor to obtain high permeability, the space inside said layer of loading material not being entirely taken up by said conductor, whereby the conductor has room for expansion during the heat treatment.
35. 10. The combination with a copper conductor of a layer of magnetic material thereabout which is capable of having developed therein high permeability at magnetizing forces encountered in signaling, but which has to be heat treated after being applied to the conductor to obtain high permeability, the loading layer fitting the conductor loosely, whereby the conductor has room for expansion during the heat treatment.
40. 11. The combination with a signaling conductor, of a layer of hardened wire or tape laid spirally thereon to increase the inductance, said wire or tape being of an alloy which is capable of having high permeability developed therein by heat treatment.
45. 12. The combination with a signaling conductor, of a non-adherent layer of hardened alloy formed over said conductor to increase the inductance, said alloy consisting chiefly of nickel and iron.
50. 13. The combination with a signaling conductor, of a layer of hardened wire or tape laid spirally thereon to increase the inductance, said wire or tape being of an alloy consisting chiefly of nickel and iron.
55. 14. The combination with a conductor, of a layer of magnetic material thereabout the permeability of which is more sensitive to strain than that of iron and which is capable of having developed therein high permeability at magnetizing forces encountered in signaling, but which has to be heat treated after being applied to the conductor to obtain high permeability, the inner surface of said loading material being retained out of forcible contact with the outer surface of said conductor in such manner as to relieve or prevent strains which would materially lower the permeability.
60. 15. The method of continuously loading a signaling conductor with magnetic material capable of having higher permeability than iron developed therein at magnetizing forces encountered in signaling, which comprises hardening the material, surrounding the conductor with a layer of the material in hardened form, heating the loaded conductor to a temperature below the melting point of the conductor and cooling it.
65. 16. The method of continuously loading a copper signaling conductor with magnetic material consisting chiefly of nickel and iron, which comprises hardening the magnetic material, surrounding the conductor with a layer of the material in hardened form, heating the loaded conductor to a temperature below the melting point of the

- conductor and cooling it, a portion of the cooling being at a rate greater than an annealing rate and which will develop higher permeability in the loading material than 5 an annealing rate.
17. The method of continuously loading a signaling conductor with magnetic material which comprises forming the material into a wire, alternately annealing and reducing 10 the diameter of the wire by drawing, subsequently forming the wire into a tape and trimming the edges to produce a tape of uniform width, the final stage before trimming being one of mechanical working to 15 harden the tape, and winding the tape spirally upon the signaling conductor, with slight spacing therebetween.
18. The method of preparing magnetic material for inductive loading which comprises alternately annealing and reducing 20 the thickness of the material by mechanical working, the final stage being one of mechanical working sufficient to reduce the thickness by at least one-half the thickness of the finished material.
19. The method of preparing nickel-iron alloy for inductive loading which comprises alternately annealing and reducing the thickness of the material by mechanical working, the final stage being one of mechanical working sufficient to reduce the thickness by at least one-half the thickness of the finished material.
20. The method of continuously loading a signaling conductor with nickel-iron alloy which comprises alternately annealing and reducing the thickness of the alloy by mechanical working, the final stage being one of mechanical working sufficient to reduce the thickness by at least one-half the thickness of the finished material, subsequently applying the alloy to a signaling conductor, and heat treating the alloy on the conductor.

In witness whereof, I hereunto subscribe my name this 26th day of April A. D., 1922.

GUSTAF W. ELMEN.